

# UNITED STATES PATENT OFFICE.

THOMAS BOLAS, OF CHISWICK, ENGLAND, ASSIGNOR TO SELF-DEVELOPING PLATE COMPANY LIMITED, OF HOLBORN, ENGLAND.

## MANUFACTURE OF CELLULOID OR THE LIKE.

964,483.

Specification of Letters Patent. Patented July 19, 1910.

No Drawing.

Application filed October 3, 1908. Serial No. 456,084.

*To all whom it may concern:*

Be it known that I, THOMAS BOLAS, a subject of the King of Great Britain, residing at 60 Grove Park Terrace, Chiswick, in the county of Middlesex, England, have invented certain new and useful Improvements in the Manufacture of Celluloid or the Like, of which the following is a specification.

This invention relates to an improved method of manufacturing pyroxylin in a transparent condition in sheet form, the pyroxylin being for the purposes of this invention so completely gelatinized by the use of a suitable solvent that the sheet will, on drying, become compact, structureless or fiberless and transparent.

The present invention has for its object the formation and mode of using a sheet or sheets of pyroxylin so completely gelatinized by a suitable solvent that the structural or fibrous character thereof is lost or destroyed; a compact transparent sheet of pyroxylin suitable for use as a base for photographic emulsion being obtained by means involving far less expenditure of solvent than obtains when films or sheets are made by casting or flowing with a solution of pyroxylin. Further, in many cases there is a saving of labor and consequent cost in the process of manufacture with the advantage of a superior product; a product which is harder, more elastic, and more inert chemically than the usual sheets or films of celluloid sold for photographic purposes—which ordinarily contain much camphor.

I am aware of many early attempts to industrially realize the agglomeration of pyroxylin into a compact mass but all these differ in essential features from the present invention. Thus for example at one of the Cantor lectures delivered by the present applicant before the Society of Arts on the 30th February, 1880, there were displayed and described several samples of celluloid articles which had been formed by pressure from pyroxylin that had been moistened with a solvent, and in the printed version that appears in the "Journal of the Society of Arts" dated the 27th August, 1880, it was stated:—

"Another celluloid-like body, due to the ingenuity of Mr. Parkes, of Birmingham, is obtained by softening nitro-cellulose by means of alcohol and forcing the product into molds. This substance is exceedingly tough, while it has the advantage of being

free from camphor, and is capable of resisting the action of heat to a considerable extent."

There have been and are many uses of sheets of complete or made celluloid softened by a solvent, but these uses are extraneous to my invention as I employ a solvent to gelatinize an original sheet of nitrated fibrous material and thus to give it for the first time its celluloid-like compact or impervious character. In short I do not soften a sheet of celluloid-like material by my softening or gelatinizing process, but I produce the celluloid-like character of my sheet pyroxylin by the use of an amount of high or complete solvent insufficient to dissolve the material, and at the same time I retain the sheet like form; this change it will be noted is effected by the solvent independently of any kneading stress or pressure.

The purification or treatment of masses or grains of pyroxylin, by the action of a partial solvent or a solvent mixed with an inert fluid, is known to me but this in no way bears on the present invention as my method only applies to sheets of the original nitrated material retaining the original form, and, as will be realized from the description hereinafter given, my invention is only applicable to sheets, and indeed to sheets of very thin substance. Moreover my method requires complete or perfect solvents used in moderate quantity or in quantity insufficient to totally dissolve the solid, the practical problem in the successful working of my method being to produce the maximum of gelatinizing effect with a minimum of solvent this being applied by spraying, flowing or the like. It has also been proposed to use a solvent on compressed masses of nitro-cellulose to harden and varnish the surface. Here again however the process is quite distinct from mine, which depends on the use of uniformly thin sheets, and complete or thorough gelatinization by the solvent.

The raw material or sheet cellulose having been nitrated in a usual manner by a mixture of acids is subsequently gelatinized. For the purposes of my invention the said material should be thin, even in texture, and as pure chemically as possible. It may be paper, linen, cotton cloth, papyrus or the like, but of all the materials hitherto used I

prefer the "chemically pure filter papers" as sold for laboratory use, as, for example, the pure white English filtering paper mill No. 633 which has given highly satisfactory results, the thickness being such that a sheet 24 inches square weighs about 333 grains, corresponding to 20 lbs. to the ream or thereabout. I do not however confine myself to this weight as I have used with equal success a similar paper of five times the weight and heavier paper may even be employed, but from the point of view of rapid and easy nitration followed by rapid action of the solvent I usually prefer a thin paper, often thinner than that mentioned, and the combining of several or many layers of the nitrated paper before or after gelatinization by a solvent is expedient when I require a thick product; with thinner paper than that mentioned above, as, for example, tissue paper, the result is good by reason of rapid and complete nitration but extremely thin paper is inconvenient to handle. The paper, which should be in a completely dry state, is now immersed in or slowly passed through a nitrating mixture of the known kind, such as a mixture of nitric acid and sulfuric acid or of sulfuric acid and nitrate of potash or nitrate of soda. As an example I give the following: sulfuric acid, of specific gravity 1.843, one volume; nitric acid, of specific gravity 1.42, one volume.

On mixing, the temperature rises somewhat; ordinarily to 120° Fahr. or 130° Fahr. and the mixture may be used at this temperature or it may be allowed to cool. The paper is now passed or drawn slowly through the mixed acids, a course which would naturally be followed in working with a roll or reel of the paper. When, however, sheets are being employed it will generally be convenient to immerse the sheets completely. Three minutes in the acid mixture may be sufficient for the thin (20 lb.) paper mentioned above, but longer is desirable as giving a more glass like and clear product. Ordinarily the paper may remain in the acid mixture for twelve hours or more without harm resulting, but speaking generally the best time of immersion is from ten to fifteen minutes for 20 to 30 lb. filtering or blotting paper of the kind referred to; harder or thicker material will require longer. Should opalescent or whitish patches show when the solvent has acted on the nitrated paper the indication is that of insufficient nitration.

On removal from the acid mixture the nitrated cellulose or pyroxylin, whether in the form of a band or sheets, is well washed, and an alkaline addition may be made to the wash waters; when the water has been dried off or removed, say, by soaking in alcohol, by exposure to the air or by heat or in any other well known way, the said paper is

fully saturated by spraying, flowing or a similar procedure with a solvent of pyroxylin so that the solid material becomes completely gelatinized or structureless, but this must be accomplished upon or in close proximity to a support so that the gelatinized sheet shall not be deformed or strained. This supporting of the gelatinized sheet is necessary to the success of the treatment, but it is to be understood that no particular means of supporting are to be regarded as forming part of this invention. When sheets of nitrated cellulose (sheets as distinguished from a band) are being treated the support ordinarily used is a slab of glass, 70 marble or other convenient or like material. This slab may be rubbed over with French chalk to diminish any subsequent tendency to adhesion, it is then leveled, flooded with a thin layer of the solvent and the sheet of 75 nitrated cellulose is laid upon the layer of solvent which now penetrates and gelatinizes the sheet. When dry the celluloid like and transparent sheet of pyroxylin is removed or peeled away from the support. 80 When a celluloid sheet, or celluloid like sheet of greater thickness is required several sheets of nitrated cellulose are laid down as a group upon the slab and gelatinized, or they may be laid down in succession on the slab, 85 the slab being again flooded with solvent before each additional sheet of nitrated cellulose is laid down. The thickened or composite sheet of pyroxylin is then allowed to dry on the slab after which the compound 90 sheet is peeled off.

When the nitrated cellulose is in the form of a roll or band, as it is gelatinized it may be received on slabs of glass or other rigid material, the solvent being sprayed or allowed to flow on the nitrated cellulose as it reaches the slab, the slab being drawn forward to keep pace with the unwinding of the roller. When, however, long bands of the product are required the gelatinized material 100 is best received on a flexible band which may be composed of metal, gelatin or the like. An alternative method is to receive the gelatinized nitro-cellulose on a warm roller from which it passes to other warm rollers 105 thereby drying and leveling it. Instead of the rollers I may employ an endless band of flexible metal or material, this being warmed by steam boxes or the like. The method of working with bands and of drying or mechanical treatment herein referred to being well known in connection with ordinary celluloid and other impervious methods no general claim is made in respect thereof; they are referred to in the present description as 110 bearing on the manner in which the herein described sheet of pyroxylin may be handled or treated before or after having been moistened with the solvent whereby it is 115 gelatinized or its fibrous structure so de- 120 125 130

stroyed as to make it compact and impervious.

When the gelatinized pyroxylin sheet is allowed to dry on the glass or other slab it 5 will generally be found on stripping or peeling off the material, that the side which has been in contact with the glass or other support is smoother than the upper or outer side. This upper side may be smoothed by 10 rolling, burnishing or calendering. If preferred the rougher side may be smoothed by flooding a plate or slab with a solvent of pyroxylin, and laying the sheet, rougher side downward on the flooded side of the slab. 15 When again dry the material is once more stripped or peeled off. Another method of smoothing the rougher surface of the pyroxylin sheet is to flood the said surface with a warm solution of gelatin while the material 20 is still on its support, and when the gelatin is dry or nearly so the film is peeled off with the stratum of gelatin still adhering to the pyroxylin and laid the gelatinized side down on the support as already described, but in 25 this case water and not a solvent of pyroxylin must be employed to soften the surface and establish adhesion between the gelatin-coated surface and the surface of the support.

30 The herein described celluloid-like film may be coated with sensitive emulsion to render it suitable for photographic purposes, the operation being performed by flowing the emulsion over the celluloid-like 35 film while on its support or by drawing the film over a roller revolving in a trough of the emulsion or in any other way known to experts.

By the term solvent of pyroxylin, I mean 40 any liquid capable of dissolving the material and I may use any one of the many simple or mixed solvents commonly employed. Ordinarily I prefer amyl acetate or a mixture of amyl acetate with acetone; with or 45 without an addition of camphor in either case. A coloring matter can be added to the solvent when a colored product is required.

It is within my knowledge that many proposals have been made for rendering blotting paper or the like translucent by various 50 agencies such as the treatment in which resinous products are incorporated, and upon which the transparency depends; also the uniting or agglomerating of sheets of nitrated

paper while in an acid bath. Such a mode 55 of procedure would, however, fail in securing the object aimed at in the present invention, viz: equal nitration, facilities for the removal of acid and complete gelatinization of the sheets by the action of a high solvent. 60

I make no general or universal claim to the use of flexible bands or sheets as supports for soft materials of the celluloid class as there have been numerous proposals in this connection. 65

As regards my use of a stratum of gelatin on my celluloid material, and the fact that this stratum of gelatin would ordinarily be at the back of my film when coated with photographic emulsion as described, I may 70 state that my object in so using gelatin is to somewhat fill or level the less even surfaces of the material, previous to the transfer in reversal above referred to. Composite films of celluloid and gelatin are well known in 75 relation to photographic uses, indeed the ordinary and well known non-curling roll film is a combination of this class and many patents have been granted relating to stratified combinations of celluloid and gelatin. 80

What I claim and desire to secure by Letters Patent of the United States is:—

1. The method of manufacturing transparent sheets of pyroxylin or the like suitable for use as a basis for photographic 85 emulsion consisting in producing a uniformly nitrated pyroxylin in sheet form, rendering the same transparent by treatment with a solvent, supporting the same until dry, then subjecting the sheet of dried 90 pyroxylin to a gelatinous solution or liquid which shall smooth or render the whole uniform, and then to reversal on the means of support for the purpose of smoothing the 95 faces of the said sheet.

2. The method of manufacturing a detached transparent sheet or film of pyroxylin suited as a base for photographic emulsion, by treating very thin nitrated material with a spray of solvent, so as to harden and 100 compact the sheet, and with the aim of producing a detached sheet.

In testimony whereof I affix my signature in presence of two witnesses.

THOMAS BOLAS.

Witnesses:

T. SELBY WARDLE,  
T. J. OSMAN.